

# UNITED STATES PATENT OFFICE

WILLIAM C. ZELLER, OF PERTH AMBOY, NEW JERSEY, ASSIGNOR TO ERNEST G. DRAPER, OF BROOKLYN, NEW YORK.

## COMPOSITION FOR FIREPROOFING MATERIALS.

1,116,349.

Specification of Letters Patent.

Patented Nov. 3, 1914.

No Drawing.

Application filed April 22, 1914. Serial No. 833,615.

*To all whom it may concern:*

Be it known that I, WILLIAM C. ZELLER, a citizen of the United States, and a resident of the city of Perth Amboy, county of Middlesex, and State of New Jersey, have invented a new and useful Composition for Fireproofing Materials, of which the following is a specification.

In these days fireproof building construction is extensively employed and in some places is required by the municipal regulations or those of fire commissioners. It is relatively easy to secure substantial non-inflammability in the strictly structural part 10 of a building, but not so easy to secure fire resisting quality in the trim, in the interior wall construction and in the fabrics employed, because although means for rendering these parts of a building non-inflammable, or at least fire resisting, have been long known, yet such treatment, so far as I am aware, has always heretofore been attended with a series of objections, among 15 which are the color given to the fireproofed article, whatever it may be, due to the fireproofing material employed, also in some instances an objectionable odor, in other instances an objectionable hardness and stiffness and in almost all instances a marked increase in cost.

After extensive experimentation I have discovered a new solution or composition of matter better adapted to the purpose above stated than any of which I am aware. Its 35 ingredients and preferred proportions are as follows: To one gallon of water which may be used hot or cold, but preferably hot, add ammonium sulfate 19 ounces, ammonium phosphate 4 ounces, sodium phosphate 1 ounce, borax 1 ounce. These chemicals as offered on the market are usually in crystal or powdered form but since they are all soluble in water it is easy to make a solution thereof.

45 The purpose or function in the mixture of the stated chemicals is as follows: Ammonium sulfate and ammonium phosphate are both good fireproofing materials. The phosphate is the better of the two because it generates in the presence of heat more ammoniacal gases than the sulfate and hence is more preventive of ignition and reduces inflammability. Its cost, however, being

several times that of the sulfate, I prefer to use them conjointly in about the proportions 55 stated, because in this way the cost of my new product is reduced and as an added advantage a bulk of fire resisting material sufficient to thoroughly impregnate the material being treated is secured, and likewise 60 owing to the increased amount, they serve also in drying out as a filler for the material, adding to its solidity and strength.

Sodium phosphate is used principally for its decolorizing effect. It seems to have 65 some chemical co-active operation with the ammonium phosphate in this respect so that the products treated by my composition, whatever they may be, are after drying out not materially changed in shade or color 70 from that they had prior to the treatment. They are thus better adapted to much interior work where light colored or delicate decoration is to be subsequently applied, as by dyeing, painting, staining and the like. 75

Borax is used to prevent discolorization due to the presence in the article or structure treated of metal, such as screws, nails, wire, piping and the like. The borax also acts as a neutralizer of the solution. 80

My new composition or solution is, as stated above, adapted to use in the treatment of wood, natural or artificial, textile fabrics, fibrous material and the like and may also be used to impregnate insulating materials 85 or articles and it is adapted to the dipping, boiling or other known process and may be used hot or cold, moderate heat at least being preferred.

The proportions given herein are not arbitrary, on the contrary may be departed from within limits and still the essential benefits of the invention be realized, the formula given above being suggested merely as a good example. 90

It will of course be understood that if my composition is presented upon the market as an article of commerce, it is immaterial whether the ingredients be dissolved and offered in liquid or paste form, or whether the chemicals named be in crystal, powdered or other dry form to be dissolved at the time of use. 100

I claim:

1. A fireproofing composition comprising 105 ammonium sulfate, ammonium phosphate,

sodium phosphate and borax, as and for the purpose set forth.

2. A fireproofing solution comprising ammonium sulfate, ammonium phosphate, sodium phosphate and borax dissolved in water, as and for the purpose set forth.

In testimony whereof I have signed my

name to this specification in the presence of two subscribing witnesses.

WILLIAM C. ZELLER.

Witnesses:

GEO. N. MENDLES,  
OLIVER A. ADOLF.